

1

3,023,103

### ANTIFOGGANTS AND STABILIZERS FOR PHOTOGRAPHIC SILVER HALIDE EMULSIONS

Fritz Dersch and Millet R. De Angelus, Binghamton, N.Y., assignors to General Aniline & Film Corporation, New York, N.Y., a corporation of Delaware  
No Drawing. Filed Aug. 2, 1960, Ser. No. 46,906  
7 Claims. (Cl. 96—109)

The present invention relates to the use of antifogging 10 and stabilizing agents for photographic silver halide emulsions.

It is known that light-sensitive emulsions such as gelatino-silver halide emulsions have a tendency to fog. This fog may be due to a number of causes as, for example, excessive ripening of the emulsion, storage of the film at elevated temperatures and humidity or prolonged development of the exposed emulsion.

A number of compounds have been described in the literature as being effective in preventing an increase in fog to thus stabilize or control the keeping qualities of the silver halide emulsion. Although many of these compounds have the ability to reduce the fog tendencies and to improve the stability of the emulsion, they are deficient in that they lower the sensitivity of the emulsions and often reduce optical and dye sensitivity.

We have now discovered that heterocyclic compounds containing a simple-5-membered nitrogenous heterocyclic ring, the 2-position of which is substituted with a guanidino radical, are not only excellent stabilizers or antifogging agents for light-sensitive silver halide emulsions but, in addition, have the faculty of performing this function without lowering the sensitivity of the emulsion with which they are associated or without reducing the sensitivity of the emulsion to light of longer wave length attributable to the presence of sensitizing dyes.

The use of such compounds to inhibit fog and to stabilize silver halide emulsions either by locating the same in the emulsion or in layers adjacent thereto or in processing baths for the emulsion constitutes the purposes 40 and objects of the present invention.

The antifoggants the use of which are contemplated herein may be represented by the following formula:



wherein X represents the radicals necessary to form a benzo ring and Y is S, O or NH.

Examples of compounds within the ambit of such formula which we have found to be effective are:

2-guanidino-benzimidazole of the following formula—



5-chloro-2-guanidino-benzimidazole

4,6-dichloro-2-guanidino-benzimidazole

5,6-dichloro-2-guanidino-benzimidazole

4,5,6-trichloro-2-guanidino-benzimidazole

5-bromo-2-guanidino-benzimidazole

2

5-nitro-2-guanidino-benzimidazole  
5-methoxy-2-guanidino-benzimidazole  
5-methyl-2-guanidino-benzimidazole  
4,6-dimethyl-2-guanidino-benzimidazole  
5-phenyl-2-guanidino-benzimidazole  
4,6-dinitro-2-guanidino-benzimidazole and the like  
2-guanidino-benzthiazole of the following formula—



and such compounds substituted in the 5-position by chloro, bromo, nitro, methoxy or methyl or in the 4,6- and 5,6-position by chloro or bromo

2-guanidino-benzoxazole of the following formula:



and such compounds substituted in the 5-position by chloro, bromo, nitro, methoxy, methyl, phenyl or in the 4- and 6- or 5- and 6-positions by chloro or bromo, and in the 4- and 6-positions by methyl.

The products utilizable herein are prepared by reaction of orthophenylenediamine-dicyandiamide with an orthophenylene-diamine (benzimidazole), with an ortho-aminobenzenethiol (benzthiazole) or with an ortho-amino-phenol (benzoxazole). The reactions are conventional and are described in the literature.

The invention will be further illustrated by the following examples in which the parts are by weight.

#### Example I

1 kilogram of a silver halide emulsion in gelatin containing 2% of silver iodide and 98% of silver bromide was prepared in a conventional manner. A 1% solution of 2-guanidino-benzimidazole was added to the emulsion as an antifoggant and stabilizer. The emulsion samples contained 0.6 mol of silver halide. The emulsion samples were coated on a suitable cellulose ester base and dried. Samples of these film coatings were then exposed in a Type IIB Sensitometer in a developer of the following composition:

|                                | Grams |
|--------------------------------|-------|
| 50 Metol                       | 1.5   |
| Sodium sulfite, anhydrous      | 45.0  |
| Sodium bisulfite               | 1.0   |
| Hydroquinone                   | 3.0   |
| Sodium carbonate, monohydrated | 6.0   |
| Potassium bromide              | .8    |
| 55 Water to make 1.0 liter.    |       |

| 60      | Quantity of compound used | Relative speed | Fog at 12' development | Fog at 6' development |
|---------|---------------------------|----------------|------------------------|-----------------------|
| 0.      | 100                       | .32            | .27                    |                       |
| 30 mg.  | 100                       | .32            | .22                    |                       |
| 60 mg.  | 100                       | .30            | .23                    |                       |
| 100 mg. | 100                       | .27            | .21                    |                       |
| 200 mg. | 100                       | .29            | .21                    |                       |
| 300 mg. | 100                       | .25            | .17                    |                       |

The 2-guanidino-benzimidazole was prepared as follows:

10 grams of orthophenylenediamine-dihydrochloride were dissolved in 100 milliliters of water. To the solution were added 10 grams of dicyandiamide and the reaction mixture heated to reflux for 5 hours. The reaction mixture was allowed to cool at room temperature and 20 milliliters of a 40% sodium hydroxide solution were added. Yellowish plate-like crystals precipitated and were chilled and collected. The solid was recrystallized from boiling water after previous charcoal treatment. The product—the pure monohydrate—melted at 237-238° C.

*Example II*

The procedure was the same as in Example I with the exception that the guanidino-benzimidazole was replaced by the same amount of 2-guanidino-benzthiazole.

The results were similar to those obtained in Example I.

The 2-guanidino-benzthiazole was prepared by dissolving 12.5 grams of ortho-aminobenzenethiol in 100 milliliters of ethanol and 40 milliliters of concentrated hydrochloric acid. 8.4 grams of dicyandiamide were added and the reaction mixture refluxed for 3 hours. The preparation was chilled in an ice bath and a white solid precipitated. The solid was collected and washed with cold water. Conversion to the free base was effected by dissolving the hydrochloride obtained above in 200 milliliters of hot water and 30 milliliters of a 40% solution of sodium hydroxide. The free base separated immediately and was collected and crystallized twice from an ethanol-water mixture after previous charcoal treatment. The product was pearly white and melted at 167-8° C.

*Example III*

The procedure was the same as in Example I excepting that the guanidino-benzimidazole was replaced by the same amount of 2-guanidino-benzoxazole.

The results were similar to those obtained in Example I.

The 2-guanidino-benzoxazole was prepared by dissolving 100 grams of ortho-aminophenol in a mixture of 100 milliliters of concentrated hydrochloric acid and 100 milliliters of ethanol. After heating to reflux for 15 minutes, 80 grams of dicyandiamide were added and the heating continued for 2.5 hours. The reaction mixture was chilled and filtered to yield a dark brown solid weighing 130 grams. Conversion to the free base was effected by dissolving 50 grams of hydrochloride in 300 milliliters of boiling water. To this were added 13 grams of potassium hydroxide in 50 milliliters of water. The base separated immediately and after cooling was filtered and washed with cool water. The product was crystallized by dissolving in ethanol and treating with charcoal. It was poured into a large volume of water and a second crystallization was effected by dissolving in boiling water. The pale yellow plates obtained melted at 183-4° C.

*Example IV*

Exposed samples of a photographic film were developed for 12 minutes at 65° F. in a standard metol-hydroquinone developer. Two tests were made, one with the normal developing solution and one with a developer containing 100 milligrams of 2-guanidino-benzimidazole per one liter of developer. Sensitometric strips, developed in the normal developer (control) for 12 minutes showed a fog of .30, whereas those strips which were developed in the developer containing the antifoggant had a fog of .20.

*Example V*

The procedure was the same as in Example IV excepting that the 2-guanidino-benzimidazole was replaced by 5-chloro-2-guanidino-benzimidazole.

The results were similar to those of Example IV.

The 5-chloro-2-guanidino-benzimidazole was prepared in the same way as the 2-guanidino-benzimidazole except-

ing that in lieu of orthophenylenediamine-dihydrochloride there was employed 4-chloro-orthophenylenediamine-dihydrochloride.

Any of the above-noted guanidino compounds may be used in lieu of those of the examples. They may be prepared by using in lieu of the orthophenylenediamine-dihydrochloride, orthoaminobenzenethiol or ortho-aminophenol, the correspondingly substituted, disubstituted or tri-substituted parent material. For example, 4,6-dichloro-2-guanidino-benzimidazole was prepared while using 3,5-dichloro-orthophenylenediamine, 5-nitro-2-guanidino-benzthiazole was prepared while starting with 4-nitro-ortho-aminobenzenethiol in lieu of the ortho-aminobenzene-thiol. Similarly, 4,6-dimethyl-2-guanidino-benzoxazole was prepared by starting with 3,5-dimethyl-ortho-aminophenol rather than the ortho-aminophenol.

Beneficial effects and fog reduction are obtained when solutions of the aforementioned compounds are incorporated in the silver halide emulsions as "ripening finals" or as "coating finals." "Ripening finals" are added during the ripening or the sensitivity increasing stage of the emulsion making process. Such additions may be made before, during or after the decomposition of the soluble silver salt such as silver nitrate by means of soluble halides such as potassium bromide in the presence of a colloidal carrier such as gelatin, PVA, solubilized casein or albumin.

"Coating finals" are added to the emulsion just prior to coating on a suitable support such as glass, paper or film at a time when the emulsion has nearly obtained its maximum sensitivity.

When used as "ripening finals," the antifoggants or stabilizers hereof are best used in a concentration of 1 to 25 milligrams per 0.6 mol of silver halide and when used as "coating finals" in a concentration of 10 to 300 milligrams per 0.6 mol of silver halide. The concentration used depends on the type of emulsion employed, and it is advisable to determine the optimum concentration from case to case. In some instances, it is advantageous to apply the antifoggant in an adjacent layer, i.e., in a separate undercoating layer or in an anti-abrasion gelatin over-coating. In other cases, desirable results accrue when they are employed in the processing baths.

The antifoggants which we utilize may be employed in various types of photographic emulsions, e.g., non-sensitized, orthochromatic, panchromatic, X-ray emulsions and color emulsions. They may be used in combination with other antifoggants and stabilizers or in combination with sulfur, reduction- and metal-sensitizers or with polyoxyethylene accelerators.

Various modifications of the invention will occur to persons skilled in the art. Thus, it is evident that in lieu of the examples any of the antifoggants specifically mentioned may be employed. We, therefore, do not intend to be limited in the patent granted except as necessitated by the appended claims.

We claim:

1. Light-sensitive photographic material comprising a base and a light-sensitive silver halide emulsion thereon, said light-sensitive material containing as an antifoggant a compound of the following constitution:



wherein X represents the atoms necessary to form a benzo radical and Y is selected from the class consisting of S, O and NH.

2. The article as defined in claim 1 wherein said antifoggant is located in the silver halide emulsion.

3. The article as defined in claim 1 wherein the antifoggant is located in a layer adjacent to the silver halide emulsion.

4. Light-sensitive photographic material comprising a base with a light-sensitive silver halide emulsion thereon, said emulsion containing as an antifoggant the compound 2-guanidino-benzimidazole.

5. Light-sensitive photographic material comprising a base with a light-sensitive silver halide emulsion thereon, said emulsion containing as an antifoggant the compound 2-guanidino-benzoxazazole.

6. Light-sensitive photographic material comprising a base with a light-sensitive silver halide emulsion thereon, said emulsion containing as an antifoggant the compound 2-guanidino-benzthiazole.

7. The process of minimizing and preventing fog in light-sensitive silver halide materials comprising a base

having a light-sensitive silver halide emulsion thereon, which comprises exposing the emulsion and developing the same in the presence of an antifoggant of the following formula:



10 in which X represents the atoms necessary to form a benzo ring and X is selected from the class consisting of O, S and NH.

No references cited.